

Patented June 4, 1929.

1,715,855

# UNITED STATES PATENT OFFICE.

FORD H. McBERTY, OF POUGHKEEPSIE, NEW YORK, ASSIGNOR TO THE DE LAVAL SEPARATOR COMPANY, OF NEW YORK, N. Y., A CORPORATION OF NEW JERSEY.

## PROCESS OF CLEANING FABRICS.

No Drawing.

Application filed May 19, 1927. Serial No. 192,794.

My invention relates to the cleansing of fabrics and more particularly to the cleaning of fabrics by the so-called dry cleaning process wherein the fabrics are subjected 5 to the action of gasoline or other solvent. In this process, the solvent, with use, becomes discolored, and it is subjected to treatment adapted to effect its decolorization. 10 While such processes are superior to older cleaning processes in important respects, it is found that, after cleaning, and particularly after cleaning several times, certain valuable qualities possessed by new fabrics 15 become lost or seriously impaired. Among these qualities are that appearance and feel known as "sheen", ability to hold a crease, and resistance to perspiration.

These qualities are dependent on the 20 fabric containing small amounts of fatty or wax-like substances.

In dry cleaning processes these substances are wholly or largely dissolved out, with the resultant loss of the desirable 25 qualities specified. It is known, however, to add to the cleaning solvent varying amounts of "soap" containing free fatty acids and fats. Since these are relatively non-volatile, they would, to some extent, remain 30 in the fabric after drying and tend to preserve, to a degree, the desirable qualities of the new fabric. The ordinary gasoline that is commonly used as a solvent also contains a small percentage of high boiling substances that would remain in the fabric after 35 drying.

Those processes, however, wherein the solvent, such as gasoline, is subjected to a decolorizing treatment are not well suited for 40 the use of cleaners' soaps or fats as additions to the solvent, because such substances are destroyed or removed by the treating agents, usually sulfuric acid and alkalies, used to dissolve color. Furthermore, the new so-called safety solvents have none of the high 45 boiling substances, and in the use of these safety solvents this possible source of substances adapted to preserve the qualities of new fabrics is eliminated.

Inasmuch as the use of safety solvents 50 and their decolorization for re-use are demanded by those engaged in commercial dry cleaning and afford, in material respects, cleaning agents of superior efficiency, it is important, if possible, to render them

incapable of destroying or seriously impairing desirable qualities of new fabrics. This is the object of my invention.

I have discovered that if a small amount of paraffin wax (between one and ten per cent) be added to gasoline or to any other equivalent cleaning solvent in which paraffin wax is soluble, it will accomplish the desired object. Paraffin wax is inert toward the chemicals ordinarily used for decolorizing the solvent. It therefore is always present in the solvent, no matter how often it has been subjected to chemical decolorizing treatments. When the fabric is subjected to centrifugal extraction, a small amount of the solvent always remains in the fabric. When this absorbed or adhering solvent contains paraffin wax, the same, or a substantial proportion thereof, remains in the fabric after the solvent has evaporated, and this wax imparts to the fabric the qualities of sheen, capacity to hold a crease and resistance to perspiration, that would otherwise be lost.

As an example of a process and apparatus 80 for dry cleaning to which my invention is applicable may be specified the process and apparatus set forth in the Flowers Patent No. 1,545,091, dated July 7, 1925.

The invention is adaptable to any cleaning 85 fluid having a boiling point that is low relatively to that of paraffin wax and in which the paraffin wax is soluble. Low boiling mineral oil hydrocarbons such as gasoline and cleaners' naphtha, coal tar derivatives such as benzol; hydrogenation solvents such as dekalin, hexalin and tetralin; turpentine; the chlorinated solvents, such as chloroform, carbon tetrachloride, tetrachlorethylene and trichlorethylene; and solutions of which any 90 low boiling hydrocarbon is a constituent: are examples of cleaning or washing solvents in which, in my process, the paraffin wax may be dissolved preparatory to using the fluid for washing.

I am aware that it is known to wash fabrics with gasoline to which "paraffin oil" has 100 been added. Such fabrics, if the oil has any substantial paraffin content, do in fact present a better appearance when fresh from the cleaning operation; but the fabric absorbs and retains the oil as well as any wax that may be in solution with the oil; and the dust and dirt catching and retaining qualities of oil are such that the fabric soils 105 110

very quickly, thereby more than neutralizing any beneficial effects which may be produced by any paraffin that may be in solution in the oil.

5 Having now fully described my invention, what I claim and desire to protect by Letters Patent is:

1. The process of cleaning fabrics which comprises washing a fabric with a solution 10 of cleaning liquid and paraffin wax.

2. The process of cleaning fabrics which comprises washing a fabric with a solution 15 of cleaning liquid and paraffin wax, expelling from the fabric a substantial proportion of the solution, and then expelling from the 20 fabric by evaporation substantially the remainder of the cleaning liquid, leaving in the fabric a substantial amount of paraffin wax.

3. The process of cleaning fabrics which comprises washing a fabric with a solution 25 of a comparatively low boiling hydrocarbon liquid constituting the major part of the solution and paraffin wax constituting a minor part of the solution.

4. A liquid for washing fabrics the dominant properties of which comprises a cleaning liquid having a boiling range not substantially higher than that of commercial gasoline.

line, the liquid carrying in solution from one 30 to ten per cent of paraffin wax.

5. The process of cleaning fabrics which comprises washing a fabric with a cleaning liquid carrying in solution not less than one per cent and not more than ten per cent of 35 paraffin wax.

6. The process of cleaning fabrics which comprises washing a fabric with a solution 40 at least ninety per cent of which comprises a cleaning fluid having a boiling range not substantially higher than that of commercial gasoline, the remaining part of the solution being principally paraffin wax.

7. The process of cleaning fabrics which comprises washing a fabric with a solution 45 of a comparatively low boiling cleaning liquid and between one and ten per cent of paraffin wax, mechanically expelling from the fabric a substantial proportion of the entire solution, and then expelling from the 50 fabric by evaporation substantially the remainder of the cleaning liquid, leaving in the fabric substantially only the paraffin wax not mechanically expelled.

In testimony of which invention, I have 55 hereunto set my hand, at Poughkeepsie, N. Y., on this 14th day of May, 1927.

FORD H. MCBERTY.